

W. J. SMART.

METHOD OF PRODUCING ORNAMENTAL SURFACES.

APPLICATION FILED FEB. 28, 1911.

1,170,567.

Patented Feb. 8, 1916.



FIG. 1



FIG. 2

FIG. 3

FIG. 4

FIG. 5

Walter J. Smart INVENTOR.  
BY Clifford E. D. ATTORNEY

# UNITED STATES PATENT OFFICE.

WALTER J. SMART, OF NEW YORK, N. Y.

## METHOD OF PRODUCING ORNAMENTAL SURFACES.

1,170,567.

Specification of Letters Patent.

Patented Feb. 8, 1916.

Application filed February 28, 1911. Serial No. 611,504.

To all whom it may concern:

Be it known that I, WALTER J. SMART, a citizen of the United States, residing in the city of New York, borough of Manhattan, county and State of New York, have invented certain new and useful Improvements in Methods of Producing Ornamental Surfaces, of which the following is a full, clear, and exact description.

10 This invention relates to surface ornamentation, particularly as applied on articles of metal, plaster and the like, to simulate materials or substances of dissimilar natures and colorings, and especially to the 15 production upon such objects of an ornamental surface of the popular and highly desirable finish commonly known as verd antique.

My invention is further designed to provide an economical, efficient and rapid method of ornamentating surfaces of metals which will withstand hard usage without losing its pleasing effects, and which when applied to plaster, or other materials of a like nature will render the same waterproof making it possible to clean the plaster object as readily as one of metal. This so-called verd antique finish as is well known, is primarily supposed to represent an old article which has been covered with verdi-gris, which by handling or rubbing has been removed from the prominent portions but remains in the crevices thereby giving a relief and high light 35 to the more prominent parts, and producing an ornamental effect. Heretofore, it has been impossible to produce a verd antique effect or finish upon plaster or similar substances, while the method of obtaining that 40 particular effect on metals has been to plate the metal with copper and apply thereto some oxidizing solution, then to immerse the article in an acid solution to cause corrosion, after which it was removed from the 45 bath and permitted to dry. Several immersions or baths were necessary to produce the desired amount of verdi-gris and the drying process consumed considerable time. After 50 drying, the process then was usually to remove with a brush the verdi-gris from the high portions and polish in some manner, as, for instance, by using a brush which had been rubbed against bee's wax. This finish, of course, being imparted by a body which 55 will melt at a low temperature, was not stable and the coating being more or less

sticky, the verdi-gris, after becoming dry, was found to often peel off with the wax. Not only is the finish above described unstable, but it is expensive and requires a 60 considerable length of time, frequently three or four days, to finish a single article.

By my improved process, the surface of the metal or plaster article to be treated, preferably one of relief and intaglio design, 65 will have applied to it a body coating or base of lacquer of any suitable coloring, and to the surface of this lacquer or base coating will be applied a second coating, preferably of a different color or of a different shade, 70 this second coating containing sufficient solvent to cause it to adhere to the body coating or base but not to coalesce therewith. In applying lacquer, which I have found it desirable to use in connection with my im- 75 proved art, I have discovered that in its usual consistency when several coats are applied, even though their application is made at considerable intervals apart, they will coalesce and will become one integral body, 80 thus differing from the action of paints or similar materials when applied in coats.

With my process, the polishing and buffing above described is entirely done away with, as is also the plating and the acid treatment. By eliminating the acid treatment, of course, the intermediate waiting for chemical action to take place upon the metal is also done away with. Furthermore, my improved finish, to produce any 90 desired shade or coloring, may be applied to any desired metal and to any other surface, while, heretofore, the verd antique in particular could only be produced upon a metal which would accumulate verdi-gris, 95 or to a surface which could be plated with a metal which would accumulate verdi-gris.

In the accompanying drawings, which illustrate the application of my invention to a piece of statuary, Figure 1 shows one of the methods, which may be employed for spraying the coating upon the object under treatment. Fig. 2 is a diagrammatic view of the base material of the object. Fig. 3 is a similar view showing the base coating of my process applied to the base material of the object. Fig. 4 is a diagrammatic view showing the second or film coating applied and Fig. 5 is a similar view after portions of the second or film coating have been removed, 105 particles of the latter remaining in the intaglio parts of the object.

In carrying out my invention, which for the purpose of clearness, I will describe with reference to its particular application for the production of the verd antique finish although any other finish or simulation may be as efficiently obtained, I apply to the article *a* under treatment a base or body-coat of lacquer-enamel *b* which is a material made from pigments ground in lacquer instead of in the customary oils or varnishes, the lacquer enamel being sprayed upon the surface of the article being treated, preferably from an atomizing device such as shown at *c*, the color employed being that which will simulate the particular metal or the like which it is desired to reproduce or imitate; for instance, when it is desired to imitate bronze, a French buff is used. In some instances it is desirable to cover the surface with a coat of clear lacquer to insure adhesion before applying the pigment lacquer-enamel. After the base-coat or body-coat of clear lacquer or priming coat has been applied, the desired number of coats will be applied to give a body-color-coat of the proper density. The article may then be permitted to dry over night in the atmosphere or may be dried in a much shorter time by artificial heat.

When the base coating has become thoroughly dry and the material hardened, I spray upon the surface to be ornamented, preferably by means of an atomizer producing a fine spray, a color such as light green or other shade which will serve to simulate verdi-gris, as designated by *d*. In applying this second coat of lacquer, which is produced with a solvent similar to that used in the production of the lacquer for use as a body coat, an atomizer is employed which is of a type to produce a very fine spray, the same being held at a considerable distance from the object or article under treatment, (see Fig. 1) so that in the spraying of the lacquer through the atmosphere from the nozzle of the atomizer to the surface of the object, a partial volatilization of the lacquer will take place and it will be deposited upon the surface of the object or article in a semi-dry or creamy state. This second or film coat will consequently adhere to the base coating previously applied to the object but will not coalesce therewith. In this connection it may be stated that where paints are applied in layers of several coats, each coat retains its individuality and does not amalgamate with the preceding coat, whereas lacquer, enamels, etc., under ordinary conditions of use, have peculiar properties or constituents, which cause coalescence of the several coats applied to a surface. Therefore, in carrying out my process and in order to make the same a practical success, it was incumbent upon me to find some method of applying a second coat of

lacquer, which would eliminate any possibility of coalescence of the second coat with the base coat and permit the ready removal of the second coat from those portions of the object which were to be so treated. This I was enabled to accomplish by spraying the second coat upon the base coat in the manner just described, whereby the volatile solvent in transit through the atmosphere from the sprayer to the surface under treatment is partially vaporized, the globules of the lacquer or pigment retaining just enough solvent to give them a sufficient consistency to cause adhesion thereof to the surface under treatment. The second coat applied in this manner, it will be observed, therefore, does not contain a sufficient amount of solvent to permit coalescence of the second coat with the base coat as would otherwise be the case and results in the deposit of a dusty film-like covering upon the surface of the object under treatment, which may be removed with comparative facility from such portions of the object as may be desired by the employment of spirits of turpentine without affecting the base or body coat, as is hereinafter more fully explained.

The spraying of the second or verd coat upon the article will build up a film of the desired coloring which will cover the entire surface with a like density. To remove the film of verd lacquer usually the relief only, I find it undesirable to use a solvent of lacquer, owing to the fact it would loosen or soften the under-coat and make an unsightly piece of work. Furthermore, it is not feasible to grind or buff off this film by ordinary means. Therefore, it is necessary to use some suitable cutting material, and I have found that turpentine, used in connection with some friction producing rubbing material, as felt for instance, possesses peculiar properties and when applied to the portions under treatment, the friction produced by rubbing will remove the film-coat from the projecting portions without injuring the under-coating, thereby uncovering the base coat representing the metal or the like and producing the high lights which are desired, the verd remaining in the intaglio as indicated at *d* in Fig. 5, the surface of the under-coating in this manner not being affected by the turpentine and the material which is used to apply it owing to the application of the verd coat in a semi-dry state. In some instances the palm of the hand and fingers may be employed for relieving the verd material. When the verd has been removed from the relief the surface may be cleaned, as for instance, by rubbing with a cloth and the coating permitted to become thoroughly hard and dry. It may then be brushed with a stiff brush, which will add to the polish on the relief portions and give it the desired luster. By

the employment of my process it will be seen that a few hours only are required for the production of a surface effect which by former methods required several days and 5 in the case of some substance could not be produced at all.

While, as before stated, I have described my invention with reference to the production of a verd-antique surface, I would have 10 it expressly understood that my process may be applied with equal facility and efficiency in obtaining any finish or representation and that such changes as may be made in practising my improved method and in the 15 new product are within the scope of my invention.

Having described my invention, I claim:

1. The method of producing ornamental surfaces simulating metal on objects of a plastic material having an intaglio and relief design, which consists in spraying on the surface of the object, a base coat of lacquer of a color simulating a metal, then spraying over the body coating a second or film coat 25 of lacquer in a manner whereby partial volatilization of the second coat will occur in transit and the lacquer will be deposited upon the object in a semi-dry state to represent a state of corrosion of the metal simu- 30 lated by said body coating, then removing

said second coating from portions of the object by the application of a cutting material thereto, and then subjecting the entire surface of the object to a polishing process.

2. The method of producing ornamental 35 surfaces on objects to simulate a metal, which consists in spraying on the surface of the object, a base coat of lacquer to represent the metal, then applying to the base coating a film coat of lacquer by spraying 40 the lacquer upon the object from a distance, whereby partial volatilization of the lacquer solvent will be effected in transit and the lacquer deposited upon the surface of the object in a semi-dry state, said second coat- 45 representing a state of corrosion of the metal simulated by the base coat, then removing said film coating from portions of the object by applying turpentine thereto and creating friction by rubbing and then 50 subjecting the entire surface of the object to a polishing process.

In witness whereof I have hereunto set my hand in the presence of two subscribing witnesses.

WALTER J. SMART.

Witnesses:

A. L. BENASARAF,  
A. G. KANE.

Copies of this patent may be obtained for five cents each, by addressing the "Commissioner of Patents, Washington, D. C."